

May 30, 1933.

L. J. LERIO, JR

1,911,696

TURPENTINE CUP

Filed Jan. 29, 1932

Fig. 1.



Fig. 2.



Fig. 5.



Fig. 3.

Fig. 4.



Inventor

L. J. Lerio, Jr.

By

E. H. Bond

Attorney

Patented May 30, 1933

1,911,696

# UNITED STATES PATENT OFFICE

LOUIS J. LERIO, JR., OF MOBILE, ALABAMA, ASSIGNOR TO THE LERIO PATENT CUP COMPANY, OF MOBILE, ALABAMA

## TURPENTINE CUP

Application filed January 29, 1932. Serial No. 589,569.

This invention relates to turpentine cups and one object of the invention is to provide a cup of the character which while similar in construction to cups now in use is free from objections which develop after a cup has been in use for a short time.

At the present time turpentine cups in general use are formed of galvanized iron but have been found unsatisfactory as the thin galvanized coating on the base metal is so thin that it wears off and decomposes due to certain acids in pine gum mixed with rain. The base metal then rusts and if a rusty cup is used, the rust mixes with the gum, discol- 15 oring the same and materially lowering the value of rosin made from the gum.

Therefore, one object of the invention is to provide a turpentine cup which may be made of galvanized iron and therefore cheaply manufactured, but has its inside coated by a layer of metal which is not affected by acids in the gum and serves to prevent the zinc coating of the galvanized iron from being eaten away and exposing the base 25 metal which will rust.

Another object of the invention is to coat the cup with a metal having a melting temperature lower than zinc used for coating galvanized sheet iron, thereby permitting the 30 inside of the cup to be coated by a hot dip process and the coating of protecting metal applied without causing the zinc coating to melt and run off of other portions of the cup.

Figure 1 is a side elevation of my improved 35 cup.

Figure 2 is a top view of the same.

Figure 3 is a section on the line 3—3 of 40 Figure 1.

Figure 4 is a section on the line 4—4 of Figure 5.

Figure 5 is a view of the blank.

Like numerals of reference indicate like 45 parts in the different views.

In accordance with this invention a tur- 50 pentine cup is manufactured in accordance with the present practice and is made from galvanized sheet iron. Galvanized sheet iron is covered with zinc and no way has been found to apply more than two ounces per square foot. Therefore, the zinc coating

is very thin and is quickly eaten away by acids in the gum so that after a short time the base metal is exposed and rusts with the result that the rust becomes mixed with gum caught in the cups and causes the gum to 55 turn dark. Also the cups soon rust to such an extent that holes are formed and the cups must be discarded and replaced by new ones.

After the cups have been formed from blanks of galvanized sheet iron the insides 60 are to be coated with a protecting coating of metal which may be pure lead, pure tin, or an alloy of lead and tin. This metal is melted and applied by a hot dip process and is applied directly to the zinc coating of the 65 galvanized sheet iron. Since zinc melts at a temperature of 787° and the metal forming the protecting coating melts at a temperature of 675° this metal can be applied without melting the zinc and since it has an af- 70 finity for the zinc it will firmly adhere to the zinc and not flake off when it cools. Ap- proximately six ounces of the lead and/or tin as alloy per square foot can be applied and therefore the protecting coating will be quite 75

thick. Since only the inside of a cup need be covered with the protecting coating, the cost of a finished cup is only slightly greater than 80 cups now in use which are formed of gal- vanized sheet iron but the coating will pre- 85 vent the gum from contacting with the zinc and therefore the zinc will remain intact and the cup cannot rust and cause the gum to turn dark. It will thus be seen that the pro- 90 tecting coating not only prevents gum turn- 95 ing dark, but also preserves the zinc coating and prolongs the life of the cup.

While it has been stated that the protect- 90 ing coating is to be applied to the inside of a cup it will be understood that the apron and other portions of a cup may be coated if so desired.

The blanks may be coated before forming the cup, the coated side, of course, to be the 95 inside of the cup.

In the drawing 1 indicates the cup.

2 designates the outer face thereof.

3 designates the coating upon the inner 100 face of the cup.

What is claimed is:

1. A turpentine receptacle formed of galvanized sheet metal and having the inside coated with metal unaffected by acids in 5 gum.
2. A turpentine cup formed of galvanized metal, and having portions with which gum contacts coated with lead.
3. A turpentine receptacle formed of galvanized metal and having the portion with 10 which the gum contacts coated with an alloy of lead and tin.
4. A turpentine receptacle formed of galvanized metal and having the portion with 15 which the gum contacts shielded by a protecting coating of metal proof against acids in gum and having a melting point lower than that of zinc used for galvanizing the base metal.
- 20 5. As an improved article of manufacture, a turpentine cup of galvanized metal provided with an inner coating embodying lead and tin of a nature to prevent discoloration of the material contained therein.
- 25 In testimony whereof, I affix my signature.

LOUIS J. LERIO, JR.

30

35

40

45

50

55

60

65